

April 3, 1934.

E. WITTCOFF

1,953,697

IMITATION STRAW HAT AND IN THE METHOD OF PRODUCING THE SAME

Filed May 20, 1933



*Fig. 1.*

*Fig. 4.*



*Fig. 1a.*



*Fig. 2.*

*Fig. 5.*



*Fig. 6.*

*Fig. 3.*



*Fig. 6a.*

INVENTOR

Edward Wittcoff.

By Ralph H. Smith  
ATTORNEY

## UNITED STATES PATENT OFFICE

1,953,697

IMITATION STRAW HAT AND IN THE  
METHOD OF PRODUCING THE SAMEEdward Wittecoff, University City, Mo., assignor  
to Caradine Hat Company, St. Louis, Mo., a  
corporation of Missouri

Application May 20, 1933, Serial No. 671,974

12 Claims. (Cl. 2—193)

This invention relates generally to the manufacture of hats and has more particular reference to an imitation straw hat and to the method or process of producing the same.

5 My invention has for its prime object the production economically, from a woven paper-strand hat-body, of a strong, durable, inexpensive, and substantially water-proof hat having a unique and attractive lustre and color and imitatively 10 resembling a genuine straw hat.

In the accompanying drawing,—

Figure 1 shows a woven paper-strand hat-body in its rough or original state or condition;

15 Figure 1a is an enlarged fragmental view of the woven paper-strands of the hat-body of Figure 1;

Figure 2 shows the hat-body at the conclusion of the first step of the process, wherein the rough hat-body is given a preliminary shaping;

20 Figure 3 illustrates the second step of the process, wherein the shaped hat-body is dipped in a sizing solution;

Figure 4 shows the sized hat-body at the conclusion of the third step of the process, wherein the dipped hat-body is dried and when dry is 25 trimmed and blocked or molded to its final desired shape;

Figure 5 represents the fourth step of the process, wherein the sized and blocked hat-body 30 is sprayed or otherwise coated with a surface finish for proofing the same against the elements and imparting a desirable color and lustre to the hat;

Figure 6 shows the finished commercial hat into 35 which the raw hat-body of Figure 1, processed through the several steps mentioned, has been converted; and

Figure 6a is an enlarged fragmental view of the woven paper-strands of the finished commercial 40 hat of Figure 6.

Referring now more in detail and by reference characters to the drawing, A designates a woven paper-strand hat-body in the raw or original condition in which it is received from the manufacturer, and it may be stated that the hat-body A is rough in appearance, with more or less widely spaced strands, unattractive in color and lustre, soft and pliable and lacking the stiffness and durability requisite for satisfactory wearing qualities, readily absorbs moisture, and merely approximately conforms to the desired shape and contour of the finished hat.

Now, in accordance with my invention, the hat-body A is first subjected to pressure in a suitable mold or die, and thereby given a preliminary

shaping or blocking, the hat-body B, as blocked, being preferably formed with a longitudinal crown-ridge 1 for reinforcing and strengthening the hat-structure and improving its appearance, as best seen in Figure 2.

60 The hat-body B is then dipped or immersed in a suitable sizing solution or substance 2 for imparting to the hat-body the stiffness and strength requisite for retaining its shape, this stage or step of the process being represented in Figure 3. 65 Preferably the sizing solution 2 is of the cellulose-gum type and comprises a collodian varnish, as pyroxylin, combined with a suitable gum, as dammar, and a solvent as ethyl acetate, mixed in the following approximate proportions, by weight, 70 namely, pyroxylin 20%, ethyl acetate 40%, and dammar solution 40%. The solution 2 is hence substantially a lacquer which readily permeates into the hat-body and penetrates both into the pores of the hat material and into the strand interstices. More or less of the ethyl acetate solvent may be employed for obtaining the desired 75 or more suitable viscosity or liquidity of the solution, as may best serve the purpose of impregnating the hat-body with the lacquer solution. 80

The dipped hat C is removed from the sizing solution 2 and then dried in any suitable manner or by any convenient means, the absorption of the sizing by the paper strands giving a flat finish 85 to the hat-body and the weaving of the strands being readily discernible, as seen at 3 in Figure 4.

The rough edge of the brim of the so treated hat-body is then trimmed, folded over, and sewed, as at 4, and the treated hat-body is then subjected to pressure in a suitable mold or die for 90 imparting to the hat-body its final shape and contour, the stiffening crown-ridge 1 being preferably further accentuated in the finally blocked and shaped hat-body D, as best seen in Figure 4.

95 The sized and blocked hat-body D is then sprayed with a finish-lacquer 5 also preferably of the cellulose-gum type comprising a vehicle of pyroxylin and dammar solution in ethyl acetate, to which is added such a substantial proportion of so-called inert or filler substances, as zinc oxide, lithopone, and titanium oxide, and to which is also added a stabilizing agent, as picric acid, as to provide on the surface of the hat-body a sufficiently dense and opaque coating of a pleasing, preferably white color. The lacquer 100 5, by reason of the pigments therein, forms on the hat-body a tenacious coating which is substantially impervious to moisture and the action of the elements, which largely fills the interstices of the paper weaving, and which forms a glossy, 105 110

- smooth, and even surface on the sprayed hat-body E, as best seen in Figure 5. More specifically, it may be stated that the finish-lacquer or spray 5 comprises the ingredients named in approximately the following proportions, namely, zinc oxide, one pound, lithopone, one pound, titanium oxide, one pound, pyroxylin, one pound, dammar solution, four pints, ethyl acetate, four pints, and picric acid, one and twenty-eight hundredths grams per gallon.
- The sprayed hat E is then permitted to dry, and when dry the hat E is strong, durable, and water-proof, may be readily cleaned by washing with water, and is of unique and pleasing color and glossy, opaque finish, resembling in large degree a genuine straw hat, its more or less open weaving being clear and distinct and, while effectively shedding water, permitting the entrance of air for ventilation.
- The sprayed hat E is then equipped with the usual trimmings as an exterior hat-band 6 and an interior sweat-band (not shown), the finished hat F being then immediately available for consumer use.
- By reason of the cheapness of the raw hat-body A and the economy of my process by which the hat F is produced, the hat F may be produced to sell at a price much less, so far as I am aware, than hats of other materials possessing comparable characteristics.
- It will be understood that changes and modifications in the several steps of the process, the composition of the several solutions employed, and the shape and contour of the finished hat may be made and substituted for those herein shown and described without departing from the nature and principles of my invention.
- Having thus described my invention, what I claim and desire to secure by Letters Patent is,—
1. An imitation straw-hat comprising a woven paper-strand body stiffened and water-proofed by a permanent surface coating of cellulose-gum lacquer.
  2. An imitation straw hat comprising a woven paper-strand body stiffened by a sizing coating of cellulose-gum lacquer and further stiffened and water-proofed by an overlying permanent surface coating of a second cellulose-gum lacquer.
  3. An imitation straw hat comprising a woven paper-strand body stiffened by a sizing coating of a transparent cellulose-gum lacquer and further stiffened and water-proofed by an overlying permanent surface coating of opaque cellulose-gum lacquer.
  4. An imitation straw hat comprising a woven paper-strand body stiffened and water-proofed by a permanent surface coating of cellulose-gum lacquer containing a filler substance composed of zinc oxide, lithopone, and titanium oxide.
  5. An imitation straw hat comprising a woven paper-strand body stiffened and water-proofed by a permanent surface coating comprising zinc oxide, lithopone, titanium oxide, pyroxylin, dammar, and ethyl acetate.
  6. An imitation straw hat comprising a woven paper-strand body stiffened and water-proofed by a permanent surface coating comprising zinc oxide, lithopone, titanium oxide, pyroxylin, dammar, ethyl acetate, and picric acid.
  7. As an article of manufacture, a hat comprising a woven body stiffened by a sizing coating and having upon its outer surface a coating of cellulose-gum-lacquer.
  8. As an article of manufacture, a hat comprising a woven body stiffened throughout by a sizing of cellulose-gum-lacquer and having upon its outer surface a finish coating of cellulose-gum-lacquer.
  9. As an article of manufacture, a hat comprising a fabricated paper-strand body stiffened throughout by a sizing of cellulose-gum-lacquer and having upon its outer surface a finish coating of cellulose-gum-lacquer.
  10. As an article of manufacture, a hat comprising a woven paper-strand body stiffened throughout by a waterproofing material and having upon its outer surface a finish coating of waterproofing material.
  11. As an article of manufacture, a hat comprising a pressed and shaped woven body stiffened with waterproofing material and having upon its outer surface a finish coating comprising cellulose-gum-lacquer.
  12. As an article of manufacture, a hat comprising a pressed and shaped fabricated paper-strand body stiffened throughout with waterproofing material and having upon its outer surface a finish coating comprising cellulose-gum-lacquer.

EDWARD WITTCOFF. 125

- 55
- 60
- 65
- 70
- 75
- 130
- 135
- 140
- 145
- 150